

# United States Patent [19]

Timmerman et al.

[11] 3,923,505

[45] Dec. 2, 1975

[54] **RECORDING MATERIAL HAVING AN ELECTROCONDUCTIVE LAYER COMPRISING THE REACTION PRODUCT OF EPIHALOHYDRIN WITH POLYETHYLENEMINE**

[75] Inventors: **Daniel Maurice Timmerman, Mortsel; Walter Frans De Winter, Berchem, both of Belgium**

[73] Assignee: **Agfa-Gevaert N.V., Mortsel, Belgium**

[22] Filed: **June 15, 1973**

[21] Appl. No.: **370,327**

[30] **Foreign Application Priority Data**

June 16, 1972 Germany ..... 028432

[52] U.S. Cl. ..... **96/1.5; 117/201; 117/218; 252/500; 260/2 BP**

[51] Int. Cl.<sup>2</sup> ..... **G03G 5/04**

[58] **Field of Search** ..... 96/87 A, 114.2, 1.5-1.8; 117/201; 218; 162/138; 252/500; 260/2.1 R, 2 BP

[56] **References Cited**

UNITED STATES PATENTS

3,210,299 10/1965 Hagge et al. ..... 260/2.1 R

|           |         |                     |           |
|-----------|---------|---------------------|-----------|
| 3,479,215 | 11/1969 | Cavagna et al. .... | 117/201   |
| 3,640,766 | 2/1972  | Jursich et al. .... | 117/201   |
| 3,642,663 | 2/1972  | Greer. ....         | 252/500   |
| 3,784,489 | 1/1974  | Dales et al. ....   | 260/2.1 R |

*Primary Examiner*—Roland E. Martin, Jr.

*Assistant Examiner*—Judson R. Hightower

*Attorney, Agent, or Firm*—William J. Daniel

[57] **ABSTRACT**

Recording materials are described comprising a support of paper or of synthetic polymer and an electroconductive layer coated on at least one side of the support. This electroconductive layer has a surface resistance lower than  $10^{11}$  Ohms/sq. and consists of or includes a major proportion of a polymer resulting from the reaction of epihalohydrin with polyethylenimine in the presence of an organic tertiary amine. This polymer is soluble in water and is rendered insoluble by heating at about 100°C. The electroconductive layer may be used as an antistatic layer in a photographic silver halide recording material. When covered with a photoconductive coating the material may be used in electrophotographic recording. With an insulating layer applied thereon, the material may be used for electrographic recording.

**9 Claims, No Drawings**

RECORDING MATERIAL HAVING AN  
ELECTROCONDUCTIVE LAYER COMPRISING  
THE REACTION PRODUCT OF EPIHALOHYDRIN  
WITH POLYETHYLENEMINE

The invention relates to a recording material comprising a support of paper or of synthetic polymer, at least one surface of which is coated with a layer that may function as an electroconductive or as an antistatic layer.

Electroconductive substances are used in recording materials to carry off static charges. For instance, it is known that in normal photographic silver halide emulsion materials the usual synthetic film supports possess the property of being charged electrostatically, whereby the charged films strongly attract the surrounding dust and thereby become soiled at their surface. Moreover, latent discharge images on silver halide emulsions, which are applied to such film supports become visible upon development. Such an electrostatic charging is caused by quickly moving the film support or light-sensitive photographic material during rolling or unrolling in the coating, cutting, or packing machines and by making the film run through the camera and the projector. It is also known that the static charging can be reduced by coating the synthetic resin support with a conductive auxiliary layer.

In other recording materials such as for use in electrostatic printing an electrostatic charge is imparted to paper or other dielectric support in a predetermined pattern. The support is conductive or must be coated with a conductive layer. For instance, in an electrophotographic recording element a photoconductive layer stands in contact with an electroconductive layer or sheet, the latter being present for carrying off the electrostatic charges at the areas of the photoconductive layer undergoing an exposure to light rays.

In electrographic materials comprising an insulating layer whereon an electrostatic charge pattern is built up by image-wise or record-wise charging, e.g., by means of a modulated electron beam, the conductive element (support or layer) serves to apply a voltage thereto, thus making possible the formation of the electrostatic charge pattern applied to the insulating top layer.

In the following description and claims the general term "recording material" is intended to include the materials used in photographic processes and in electrographic and electrophotographic processes, for which applications the surface resistance of the electroconductive layer must not be higher than  $10^{11}$  ohms per sq. at 15% of relative humidity, although according to NAKAO, SAKOMOTO, and KATAGIRI at page 105 of the Preprints of the TAPPI, First Reprography Conference at St. Charles, Ill., U.S.A., 1971 in electrophotography slight smudging of the back face of the support might already occur at resistance values higher than  $4 \times 10^{10}$  ohms/sq.

Electroconductive layers for carrying off electrostatic charges may also be useful in recording elements wherein photosensitive semiconductor compounds are activated reversibly by electromagnetic radiation and wherein the activated patterns provide irreversible images by an oxidation-reduction chemical process.

The invention provides a recording material comprising a support of paper or synthetic polymer and an electroconductive layer coated on at least one side of

said support, said electroconductive layer having a surface resistance lower than  $10^{11}$  ohms/sq. measured at 15% of relative humidity, said electroconductive layer consisting of or including a major proportion of a polymer resulting from the reaction of epihalohydrin with polyethylenimine in the presence of an organic tertiary amine, said polymer being soluble in water and becoming insoluble by heating at about 100°C.

The organic tertiary amine corresponds to the general formula:



15 wherein:  
each of  $R_1$ ,  $R_2$ , and  $R_3$  (same or different) represents an alkyl group containing up to 5 carbon atoms, a cycloalkyl group or an aralkyl group, or

20  $R_1$ ,  $R_2$ , and  $R_3$  together with the nitrogen atom represent a heterocyclic compound such as pyridine, N-alkylpiperidine, and N-alkylmorpholine.

Most suitable organic tertiary amines are trimethylamine and triethylamine.

25 Although the invention is restricted to the use of an epihalohydrin as epoxy compound, preferably epichlorohydrin, the epihalohydrin can as well be replaced by other compounds containing an epoxy group such as 1-chloro-3,4-epoxybutane, 1-chloro-1-methyl-2,3-epoxypropane, and 1-chloro-2-methyl-3,4-epoxybutane.

30 In this case the epoxy compound can be represented by the general formula:



35 wherein:  
40  $R$  is a branched or unbranched alkylene group of up to 4 carbon atoms, and  
 $X$  is a halogen atom such as chlorine or bromine. In fact  $X$  may derive from any suitable acid. However, in view of availability and better electrical conductivity the chlorine atom is used preferably.

45 The polymer directly resulting from the reaction of epihalohydrin with polyethylenimine in the presence of an organic tertiary amine is soluble in water. It becomes insoluble in water, however, when applied as a layer on a support and heated subsequently to about 100°C for a few minutes.

50 It is generally known that the polymerisation of ethylenimine does not result in a polymer that is completely composed of units having a linear structure, but that also a certain degree of branching is found. According to Zhuk, Gembitskii, and Kargin in Russian Chem. Rev. 34 (July 1965) No. 7, page 523, the degree of branching in polyethylenimine depends on the acid concentration and the temperature during polymerisation. This degree of branching may vary between 12 and 38%. The formula of polyethylenimine can be represented as follows:



wherein, depending on the degree of branching,  $x$  is comprised between 13.6 and 61.3 mole % and  $y$  between 38.7 and 86.4 mole %.

As appears from the above formula polyethylene-imine comprises primary as well as secondary and tertiary amino groups.

As generally known primary and secondary aliphatic amines in water or organic solvents and in gentle reaction conditions are converted by epichlorohydrin with a high yield according to a hydrogen substitution process into aminoalkylated compounds (Houben-Weyl : Methoden der Organischen Chemie, Makromolekulare Stoffe, Georg Thieme Verlag, Stuttgart (1961), vol. 14/II, pages 455-460).

In accordance with this reaction the primary and secondary amino groups in polyethylenimine together with epichlorohydrin in the presence of organic tertiary amines give rise to hydrogen substitution and quaternization reactions in simultaneous or consecutive processes. In the hydrogen substitution reactions the epoxy groups will react with the primary or secondary amino groups in polyethylenimine: 15  
20



wherein:  
X is a halogen atom, preferably a chlorine atom. When

halohydrin and the tertiary amine groups present in polyethyleneimine.



wherein Y is hydrogen or the group —CH<sub>2</sub>—CHOH—CH—Q with Q being X or



The compound of formula (IV) will react with a primary or secondary amino group of polyethyleneimine as described in the United Kingdom Pat. application No. 2134/72 filed Jan. 17, 1972 by Agfa-Gevaert N.V.

As a result of sterical hindrance factors the first quaternization reactions will probably occur on the nitrogen atoms of the tertiary amine



Further quaternization reactions will then occur on the tertiary amino nitrogen atoms always present as described above in the polyethyleneimine, or on the tertiary amino nitrogen atoms formed in the polyethyleneimine by the substitution reactions.

A ratio of at least 0.2 mole of tertiary amine per mole of epihalohydrin present yields - as will be proved in the Examples given hereinafter - good electroconductive polymers that can be cross-linked after a short heating at temperatures of about 100°C, whereby the electroconductivity of the polymers is preserved. One may add much larger amounts of tertiary amine to the reaction medium, even amounts of 2 moles of tertiary amine per mole of epihalohydrin, without incurring the risk that the electroconductive and cross-linkable properties of the modified polymer might be impaired sensibly. When an excess of tertiary amine in respect of epihalohydrin is present, only part of the tertiary amine joins in the quaternization reaction and the excess tertiary amine remains unmodified in solution.

These reactions are preferably performed in aqueous medium and at relatively low temperatures of about 50°C. The epihalohydrin and the tertiary amine may be mixed previously and the mixture may then be added to polyethyleneimine. However, as a result of the high reactivity of epihalohydrin with tertiary amines and in order to prevent a quaternization reaction that might immediately take place between both, the mixing and also the storage of the mixture formed has to occur at lower temperatures. Accordingly, it is much easier to mix polyethyleneimine and tertiary amine together and to add the epihalohydrin gradually to the mixture of both.

The relatively low reaction temperature of about 50°C is preferred to keep the rate of hydrolysis in aqueous medium of the epoxy groups as low as possible and to keep the degree of aminoalkylation by hydrogen substitution as high as possible. At the same time splitting off of hydrogen chloride at these relatively low reaction temperatures and re-formation of epoxygroups on the polymer are avoided. When the reaction is performed in organic medium, the danger of hydrolysis is less pronounced.

The electroconductive polymers of the invention comprise recurring units of different types. The aminoalkylated polyethyleneimine possibly comprises unsubstituted branched and unbranched ethyleneimine units as described above, and depending on the propor-

tions of epihalohydrin and tertiary amine present, recurring units of formula (I), (II), (III), (V), and (VI).

As appears from the above formulae, especially from formula (VI) the aminoalkylated polyethyleneimine comprises a certain amount of latent reaction epoxy groups and of —CH<sub>2</sub>X groups that may further react with residual primary and secondary amino groups or with tertiary amino groups respectively, to form inter-chain bridges or cross-links that will render the resulting polymer insoluble. This cross-linking can be performed easily by heating the aminoalkylated polyethyleneimine for a short period, e.g., a few minutes at about 100°C, preferably after it has been applied as a layer to a support.

The ratio of epoxy compound in respect of the amounts of polyethyleneimine and a tertiary amine has to be selected within the limits indicated above to obtain optimal properties. These properties may be summarized as follows: initially the modified polyethyleneimine has to be soluble in water and it becomes insoluble only after a simple heat-treatment. The surface resistance of a layer formed from the modified and possibly heat-treated polymer has to be lower than  $1 \times 10^{11}$  ohms/sq. at 15% relative humidity. The electroconductivity of such a layer is mainly determined by the amount of quaternized nitrogen atoms present. The higher this amount the better its electroconductivity.

The molecular weight of the polyethyleneimine before aminoalkylation with epihalohydrin in the presence of an amine has little effect on the electroconductive properties of the polymers after amino-alkylation. However, the molecular weight does affect the cross-linking reaction. The higher the molecular weight, the more efficient is the cross-linking reaction. It results from our experiments that polyethyleneimines with molecular weights ranging from 1200 to about 50,000 can be aminoalkylated. They can be applied as continuous layers to a support and the polymeric layer can easily be rendered insoluble by a simple heat-treatment.

The molecular weight of the polyethyleneimine before aminoalkylation with epihalohydrin in the presence of an amine has little effect on the electroconductive properties of the polymers after amino-alkylation. However, the molecular weight does affect the cross-linking reaction. The higher the molecular weight, the more efficient is the cross-linking reaction. It results from our experiments that polyethyleneimines with molecular weights ranging from 1200 to about 50,000 can be aminoalkylated. They can be applied as continuous layers to a support and the polymeric layer can easily be rendered insoluble by a simple heat-treatment.

Layers of the electroconductive polymeric materials can be applied from aqueous solutions by spray, brush, roller, doctor blade, air-knife, or wiping techniques to different kinds of supports, e.g., paper. Films of synthetic polymers such as cellulose acetate, polystyrene, polyester, polycarbonate, can also be coated with the electroconductive layers. If necessary, these film supports can be provided previously with a known subbing layer, whereon the electroconductive layer is coated afterwards.

When paper is used as the support, the electroconductive polymeric materials will also impart electroconductivity if the paper is thoroughly soaked with an aqueous solution of the electroconductive polymeric materials of the invention. After drying of the thus impregnated paper, the electroconductive polymeric material remains dispersed throughout the entire paper base. Electroconductivity may also be conferred to the paper base by adding a sufficient quantity of an aqueous solution of the electroconductive polymeric materials to the paper making pulp. The amount of incorporated conductive polymer is determined by the required degree of conductivity.

In all these cases the electroconductive polymer can be cross-linked and insolubilised in water and organic solvents by a simple heat-treatment e.g., by heating for a few minutes at about 100°C, whereby the electroconductivity of the polymer is not impaired. This is very

important, e.g., when a photoconductive layer of zinc oxide is applied to the electroconductive layer. Since the heated electroconductive polymer is insoluble, the photoconductive material can as well be applied thereto from aqueous or organic dispersion without fear that the electroconductive polymer would wholly or partly dissolve away.

The electroconductivity of the aminoalkylated polyethylene imines of the invention is proportional, of course, to the substitution degree of the amino groups in the polymer, to the quantity of aminoalkylated polymer present per unit of surface, and to the relative humidity of the layer. From our experiments it results that at 15% relative humidity and at about 20°C layers formed from an aminoalkylated polyethylene imine according to this invention, can easily be cross-linked and possess a sufficient electroconductivity (surface resistance lower than  $1 \times 10^{11}$  ohm/sq), when

a. during reaction between 0.3 and 1.0 mole and preferably about 0.4 mole of epihalohydrin is present per mole of ethyleneimine units in polyethyleneimine,

b. at least 0.2 mole of tertiary amine is present per mole of epihalohydrin, and

c. the layer contains at least 2 g of dry aminoalkylated polyethyleneimine per sq.m.

The electroconductivity is determined by measuring the surface resistance of layers applied to a support from a 10% aqueous solution of the aminoalkylated polyethyleneimine. The resulting layer is dried and conditioned at a specified relative humidity. The surface resistance measurements are performed by means of a cell, both poles of which have a width of 0.5 cm and are at a distance of 1 cm from each other.

These layers can only be used as an electroconductive layer in an electrographic recording element, if its surface resistance does not exceed well defined limits. The article of Nakao et al. indicated above, cites a value of  $4 \times 10^{10}$  ohm/sq as a limit for smudging of the back face of the paper support. The electroconductivity itself, however, is influenced by the degree of relative humidity. Thus it is advisable to measure a value of surface resistance at 15% of relative humidity lower than  $10^{11}$  ohms/sq. In such case a slight backmarking is unavoidable when the relative humidity is very low. The image, however, retains sufficient appeal to be commercially acceptable.

The amount of electroconductive polymeric material applied depends, of course, on the support used. When this support is made of paper and especially of a highly porous paper stock, more electroconductive polymeric material will have to be used than in the case of a non-porous synthetic support, e.g., of polyester. In general, however, an amount of 0.5 to 7.5 g/sq.m. suffices to provide the layer with a good conductivity.

In addition to the electroconductive polymer of the invention the composition of the electroconductive layer may include stabilizing agents against migrating forces, plasticizers, dispersing agents, pigments, and binders such as gelatin, starch, casein, polyvinyl alcohol and the like. It is obvious that the mixture of such

binders determinedly influences the electroconductivity of the layer. Especially gelatin is found to lower the electroconductivity of the layer much more than e.g., starch, as commonly can be found in the literature.

Moreover, the electroconductive polymers of the invention may also be combined with minor amounts, in comparison to the amount of electroconductive polymer present, of inorganic and organic salts, e.g., sodium chloride, sodium sulphate, sodium nitrate, the corresponding potassium and ammonium salts, sodium acetate, citric acid amides, hydroxypropylsucrose monolaurate, etc. These salts are known to be electroconductive. They are inexpensive but have the disadvantage that their electroconductivity is very dependent on the relative humidity. When they are combined with the electroconductive polymers of the invention, the low cost-price of these salts is linked with the excellent electroconductivity at low and high relative humidities of the electroconductive polymers.

When the electroconductive layer of the invention is to be used as an antistatic layer in a photographic silver halide recording material, the electroconductive layer is applied generally to the said sheet or web either on a surface opposite to the surface, to which the silver halide emulsion layer is applied, or as an interlayer, i.e., between the support and the light-sensitive emulsion layer or layers.

If the electroconductive layer is to be used in an electrophotographic recording material, a photoconductive coating is applied to the said polymer layer. This coating is prepared by dispersing or dissolving the photoconductive substance or substances in an aqueous or an organic solution of an insulating binder, or in a solution of such an insulating binder in a mixture of an organic solvent and water and by applying the dispersion or solution in the form of a layer to the electroconductive surface.

The electrophotographic recording element prepared with the electroconductive copolymer of the present invention is flexible and possesses a very good mechanical strength. A very good adhesion exists between the paper support and the electroconductive layer.

The electroconductive polymers may be used in combination with coatings of various inorganic as well as organic photoconductive substances such as those described in the Belgian Patent Specification 587,300, filed February 5, 1960 by Gevaert Photo-Producten N.V., the United Kingdom Pat. Specifications Nos. 964,871 filed Feb. 26, 1959, 964,873, 964,874 both filed Mar. 30, 1960, 964,875, 964,876, both filed Apr. 21, 1960, 964,877 filed May 2, 1960, 964,879 filed Apr. 26, 1960, 970, 937 filed Dec. 9, 1960 980, 879, 980, 880 both filed Feb. 17, 1961 all by Gevaert Photo-Producten N.V., in the German Pat. Specification No. 1,058,836, filed April 14, 1956 by Kalle & Co. A.G., and in the Canadian Patent Specification 568,707 of Kalle & Co A.G. issued Jan. 6, 1957. These photoconductive substances may be combined with insulating binder agents, known i.a. from the United States Pat. Specifications Nos. 2,197,552 of Joseph N. Kuzmick issued Apr. 16, 1940, 2,297,691 of Chester F. Carlson

issued Oct. 6, 1942, 2,485,589 of Frank Graz issued Oct. 25, 1949, 2,551,582 of Chester F. Carlson issued May 8, 1951 and 2,599,542 of Chester F. Carlson issued June 10, 1952, from the United Kingdom Pat. Specification Nos. 566,278 filed June 21, 1943 by Rothschild S. Slathodeon Ltd., 693,112 filed May 9, 1950 by Battelle Development Corporation and 700,502 filed Apr. 26, 1949 by Office National d'Etudes et de Recherches Aeronautiques, from the Belgian Pat. Specification Nos. 612,102 filed Dec. 29, 1961 by Gevaert Photo-Producten N.V., 711,376 filed Feb. 28, 1968, 714,257 filed Apr. 26, 1968 both by Gevaert-Agfa N.V., the French Pat. Specification No. 2,485,839 filed June 24, 1966 by Gevaert-Agfa N.V., and the Belgian Pat. Specification No. 683,145 filed June 27, 1966 by Gevaert-Agfa N.V.

Suitable dispersing agents for dispersing photoconductive materials in an aqueous medium are described in the Belgian Pat. Specification No. 703,467 filed Sept. 5, 1967 by Gevaert-Agfa N.V. and as is generally known the photoconductive substances can be spectrally sensitized as described in the Belgian Pat. Specification Nos. 708,244 filed Dec. 20, 1967 by Gevaert-Agfa N.V. and 714,258 filed Apr. 26, 1968 by Gevaert-Agfa N.V.

Photoconductive zinc oxide coatings can be successfully applied to the electroconductive polymers of the invention, especially photoconductive zinc oxide coatings with improved dark resistance and wherein the pre-exposure effect has been sharply reduced, such as described in Belgian Pat. Specification No. 612,102. Also copper(II) derivatives of aliphatic acids may be used to reduce this pre-exposure effect, e.g., copper(II) lactate, behenate, naphthenate and other copper(II) salts such as described in United Kingdom Pat. Specification No. 1,085,939.

Also mixtures of zinc oxide may be used, e.g. mixtures of small amounts of non-charge-storing zinc oxide with large amounts of charge-storing zinc oxide in order to confer to the layer an optimal height of charging. Hereby a lengthened exposure scale is obtained giving a much better tonal quality.

The aminoalkylated polyethylenimines can also very successfully be used in electrophotographic printing plates, wherein both sides of the support, which has been treated with the conductive polymer of the invention, are provided with covering layers, which prevent the solvents from impairing the support during the processing. These covering layers may contain pigments such as, e.g., zinc oxide.

The invention is illustrated by the following examples.

#### EXAMPLE 1

Solutions of 43 g of polyethylenimine in 40 ml of water and of 118 ml of a 20% by weight solution of trimethylamine in methanol were introduced in a 500 ml reaction flask provided with a stirrer, a reflux condenser cooled with a mixture of methanol and water at -20°C, a dropping funnel, and a thermometer. The mixture was cooled to 15°C.

The polyethylenimine had a branching degree of about 30%, which corresponds with the following general formula:

5



wherein  $x$  and  $y$  are 42.8 and 57.2 mole % respectively. A 10% by weight aqueous solution of this polyethylenimine had an absolute viscosity at 25°C of 8.12 cP and its viscosity number  $\eta_{sp}/c$  amounted to 0.215 dl/g for a concentration  $c$  being 1 g/100 ml.

37 g of epichlorohydrin were added dropwise in 30 minutes, causing a temperature raise of 45°C. Under permanent stirring the reaction was continued for 5 h at 65°C.

The slightly yellowish solution was cooled to room temperature and poured into 2.5 l of acetone. The tacky residue was dissolved in 200 ml of methanol and precipitated in 2.5 l of acetone and finally dissolved in 500 ml of water.

Yield: 73 g of aminoalkylated polyethylenimine. At this moment the polymer is still soluble in water, but after having been dried at 100°C it becomes insoluble in water.

#### EXAMPLES 2-11

The procedure of example 1 was repeated with varying amounts of polyethylenimine (the same as used in Example 1), epichlorohydrin and trimethylamine as starting materials. The results are given in the following table.

| Ex-<br>ample | Polyethylene-<br>imine<br>g | 20 % solution<br>of trimethyl-<br>amine in<br>methanol<br>ml | epichloro-<br>hydrin<br>g | amount of<br>modified<br>polyethyl-<br>eneimine<br>g |
|--------------|-----------------------------|--------------------------------------------------------------|---------------------------|------------------------------------------------------|
| 2            | 43                          | 59                                                           | 18.5                      | 52                                                   |
| 3            | 43                          | 73.8                                                         | 27.7                      | 64                                                   |
| 4            | 43                          | 23.6                                                         | 37.0                      | 56                                                   |
| 5            | 43                          | 59                                                           | 37.0                      | 53                                                   |
| 6            | 43                          | 177                                                          | 37.0                      | 68                                                   |
| 7            | 43                          | 236                                                          | 37.0                      | 66                                                   |
| 8*           | 2.15                        | 11.8                                                         | 3.7                       | 7.5                                                  |
| 9*           | 4.3                         | 29.5                                                         | 9.25                      | 17.5                                                 |
| 10           | 43                          | 295                                                          | 111.0                     | 206                                                  |
| 11           | 43                          | 295                                                          | 138.8                     | 234                                                  |

\*In Examples 8 and 9 the reaction occurred in sealed heavy-walled reaction tubes at 40°C for 1 h, at 50°C for another hour, at 60°C for 2 hours, and finally at 70°C for 1 hour.

#### EXAMPLE 12

Preparation of the polymer by reaction between polyethylenimine on the one hand and a cooled mixture of trimethylamine and epichlorohydrin on the other hand.

A reaction flask of 500 ml was equipped with a stirrer, a double-walled dropping funnel, a reflux condenser, and a thermometer.

The dropping funnel and the reflux condenser were cooled with a methanol/water mixture at -20°C.

In the reaction flask 21.5 g of polyethylenimine dissolved in 193 ml of water were placed.

In the cooled dropping funnel 46.25 g of epichlorohydrin and 206.5 ml of a 20% by weight solution of trimethylamine in methanol were mixed homogeneously at -10°C.

In approximately 50 minutes the contents of the dropping funnel were added to the polyethylenimine solution. Initially the temperature of the reaction medium in the flask was 24°C, but it increased slowly so as

65

to attain 40°C in consequence of an exothermic reaction. So, the reaction medium had to be cooled now and then with a water-bath of approximatively 8°C.

Subsequently the reaction medium was heated for 2 more hours at 40°C and afterwards for 4 hours at 60°C.

The clear viscous solution was poured into 3 l of stirred acetone. The precipitated polymer was washed with 1 l of fresh acetone and dissolved then in 500 ml of water.

Yield: 90 g.

10

### EXAMPLE 13

Aqueous solutions of the aminoalkylated polyethylene imines of Examples 1 to 12 were applied to a paper support in such a manner that after drying 2 g of solid product were present per sq.m. The coatings were dried at 100°C so as to insolubilize the polymer. The surface resistance values of the different samples were measured as indicated above. The results are given in the following table, wherein the abbreviations ECH, PEI, and TMA mean epichlorohydrin, polyethyleneimine, and trimethylamine respectively.

For comparison purposes was also measured the surface resistance of an uncoated paper support, of a paper support carrying a layer of pure polyethyleneimine, and of a paper support carrying a layer of polyethyleneimine that had been modified with epichlorohydrin alone according to Example 1 of the Belgian Pat. Specification No. 721,574 filed Sept. 27, 1968 by Dow Chemical Co.

15

20

25

30

pleles the proportion of moles of epichlorohydrin per mole of ethylene unit in the polyethyleneimine is greater than 0.3, but lower than 1.0 and the proportion of moles trimethylamine per mole of epichlorohydrin is always larger than 0.2.

The aminoalkylated polyethyleneimine of Example 11 in the form of a 45% weight solution in water became insoluble when stored at room temperature for 4 days.

### EXAMPLE 14

Two samples of glassine paper having a weight of 70 g/sq.m were coated with an electroconductive layer, according to the method described in Example 13 and with the aminoalkylated polyethyleneimines of Examples 1 and 4, in such a manner that after drying about 2 g of solid product was present per sq.m. For comparison purposes a same glassine paper but without electroconductive layer was used.

The electroconductive layers of both first materials and the pure glassine paper were coated with a zinc oxide dispersion prepared as follows. To 5.6 liters of dichloroethane was added 0.5 liter of GELVA MULTIPOLYMER solution RP 927A, which is the trade name of Monsanto Chemical Co. for a solution of 50% by weight of RP 927 (an insulating binder material sold for electrophotographic purposes) in a mixture of toluol, isopropanol, and ethanol (22:22:56 % by volume). To this mixture 4.2 kg zinc oxide were added. The zinc oxide used is marketed by The Durham Chemical

| Paper support                           | mole of ECH<br>mole of PEI | mole of TMA<br>mole of ECH | Surface resistance at 20°C in<br>ohm/sq (2 g/sq.m) |                       |                    | Solubility in water after<br>heating of layer at 100°C |                                |
|-----------------------------------------|----------------------------|----------------------------|----------------------------------------------------|-----------------------|--------------------|--------------------------------------------------------|--------------------------------|
|                                         |                            |                            | 15 %                                               | 50 %                  | 70 %               | After 10 min.                                          | After ½ hour                   |
| uncoated                                | —                          | —                          | $>4.2 \times 10^{13}$                              | $2.15 \times 10^{10}$ | $5.3 \times 10^8$  |                                                        |                                |
| coated with PEI                         | —                          | —                          | $>4.2 \times 10^{13}$                              | $2.13 \times 10^{10}$ | $1.93 \times 10^8$ |                                                        |                                |
| coated with PEI<br>modified with<br>ECH | 1.0                        | —                          | $2.1 \times 10^{13}$                               | $2.36 \times 10^9$    | $1.64 \times 10^7$ |                                                        | insoluble                      |
| coated with polymer<br>of example 2     | 0.2                        | 0.2                        | $1.42 \times 10^{13}$                              | $2.5 \times 10^9$     | $7.7 \times 10^6$  | insoluble but<br>swellable                             | insoluble<br>does not<br>swell |
| coated with polymer<br>of example 3     | 0.3                        | 0.25                       | $8.5 \times 10^{11}$                               | $2.36 \times 10^8$    | $8.5 \times 10^6$  | id.                                                    | insoluble<br>but<br>swellable  |
| coated with polymer<br>of example 4     | 0.4                        | 0.2                        | $3.5 \times 10^9$                                  | $8.0 \times 10^8$     | $3.86 \times 10^6$ | id.                                                    | insoluble<br>but<br>swellable  |
| coated with polymer<br>of example 5     | 0.4                        | 0.5                        | $8.5 \times 10^9$                                  | $1.9 \times 10^9$     | $7.9 \times 10^6$  | id.                                                    | id.                            |
| coated with polymer<br>of example 1     | 0.4                        | 1.0                        | $4.25 \times 10^9$                                 | $3.86 \times 10^8$    | $6.0 \times 10^6$  | id.                                                    | id.                            |
| coated with polymer<br>of example 6     | 0.4                        | 1.5                        | $1.7 \times 10^{10}$                               | $9.1 \times 10^8$     | $4.25 \times 10^6$ | id.                                                    | id.                            |
| coated with polymer<br>of example 7     | 0.4                        | 2.0                        | $5.8 \times 10^{10}$                               | $1.04 \times 10^9$    | $4.25 \times 10^6$ | insoluble but<br>but                                   | insoluble                      |
| coated with polymer<br>of example 8     | 0.8                        | 1.0                        | —                                                  | $6.8 \times 10^7$     | $2.13 \times 10^6$ | id.                                                    | swellable<br>id.               |
| coated with polymer<br>of example 9     | 1.0                        | 1.0                        | $1.77 \times 10^{11}$                              | $2.83 \times 10^8$    | $6.5 \times 10^6$  | id.                                                    | insoluble<br>does not<br>swell |
| coated with polymer<br>of example 12    | 1.0                        | 1.4                        | $4.25 \times 10^{13}$                              | $7.3 \times 10^8$     | $3.54 \times 10^6$ | id.                                                    | id.                            |
| coated with polymer<br>of example 10    | 1.2                        | 0.83                       | $2.1 \times 10^{11}$                               | $1.06 \times 10^8$    | $3.86 \times 10^6$ | id.                                                    | id.                            |
| coated with polymer<br>of example 11    | 1.5                        | 0.66                       | —                                                  | —                     | —                  | id.                                                    | id.                            |

From the above table it can be deduced that only when the paper support has been coated at a ratio of 2 g/sq.m with the aminoalkylated polyethyleneimine of Examples 1 and 4 to 8, and after heating to 100°C a water-insoluble but swellable layer is obtained, which has a surface resistance that in all circumstances of relative humidity is lower than  $1 \times 10^{11}$  ohms/sq. In these Exam-

65

Group, Birtley, United Kingdom, under the trade name ELECTROX. The resulting dispersion was ground in a sand-mill and then admixed with 1.2 liters of GELVA MULTIPOLYMER solution RP927B of Monsanto, which is the same RP927 binder material as a 50 % by weight solution in toluol. Then 1.5 liter of dichloroeth-

ane and 67 ml of a 1 % by weight solution of bromophenol blue in ethanol were added.

The coating composition formed was applied by means of a knife coater at a ratio of 30 g of zinc oxide per sq.m and dried.

The three materials were treated in a common electrophotographic copying apparatus. When the quality of copies made at different relative humidities with the materials carrying an electroconductive layer of aminoalkylated polyethyleneimine of Examples 1 and 4, are compared only slight differences can be observed. These differences are due to small changes in electroconductivity of both aminoalkylated polyethyleneimines at the different relative humidities. In the comparison material carrying no electroconductive layer considerable smudging of the back face of the support occurs at 15 % of relative humidity. This is not the case with the two other materials wherein an electroconductive layer of aminoalkylated polyethyleneimine according to the invention is present.

#### EXAMPLE 15

A glassine paper of 70 g/sq.m was coated with an electroconductive layer according to the method described in Example 13 and with the aminoalkylated polyethyleneimine of Example 5.

Upon the electroconductive layer thus formed a zinc oxide dispersion was coated that has been prepared as follows. To 500 g of toluol were added 222 g of Electrophotographic Resin EO41 solution, which is the trade name of a modified acrylic resin dissolved at a concentration of 45 % in a mixture of xylol, toluol, and n-propanol, marketed by De Soto Inc., Des Plaines, Ill., U.S.A. In this mixture were dispersed 500 g of zinc oxide type C of Vieille Montagne, Belgium, and the whole was ground in a sand-mill. Finally 5 ml of 1 % solution of bromophenol blue in ethanol were added.

The zinc oxide dispersion was applied to the electroconductive layer at a ratio of 30 g of zinc oxide per sq.m.

The material was treated in a common electrophotographic copying apparatus. Good copies were obtained, even at very low relative humidities.

#### EXAMPLE 16

To 0.807 kg of dichloroethane were added 3.670 kg of GELVA MULTIPOLYMER solution RP 927 A (trade-name) and 0.918 kg of Electrophotographic Resin EO41 solution (trade name). To this mixture 186 ml of tetrachlorophthalic anhydride as a 10 % by weight solution in ethanol and 5.56 kg of zinc oxide ELECTROX (trade-name) were added and stirred long enough to sufficiently moisten the zinc oxide pigment.

VINNAPAS UW4 (trade-name)  
dissolved in 2 liters of dichloroethane 224 g  
bromophenol blue dissolved in 70 ml of methanol 0.7 g

compound of formula:

dissolved in 34 ml of dimethylformamide compound of formula:



dissolved in 56 ml of dichloroethane 0.56 g  
copper(II) naphthenate (comprising 22 % by weight of copper) dissolved in 33.5 ml of toluene 6.7 g

VINNAPAS UW4 is the trade-name of WACKER-CHEMIE, Germany, for a high-viscous polyvinyl acetate. The dispersion thus formed was ground in a sand-mill and coated on a support of glassine paper having a weight of 70 g/sq.m. This paper had been previously coated with an electroconductive layer according to the method described in Example 13 with the aminoalkylated polyethyleneimine of Example 1 in such a manner that after drying 2 g of solid product were present per sq.m. Surface resistance at 20°C and 50 % of relative humidity of the thus covered support was  $3.86 \times 10^8$  ohm/sq.

The zinc oxide dispersion was applied to the above support in a ratio of 25 g of zinc oxide/sq.m.

The electrophotographic material obtained could be treated in full daylight conditions in electrophotographic apparatus, e.g., in a GEVAFAX 20 apparatus (trade-name of Agfa-Gevaert). Clear and contrasty copies of the original were obtained.

#### EXAMPLE 17

40 The process of Example 16 was repeated with the sole difference that in the coating composition for the zinc oxide dispersion the copper(II) naphthenate was replaced by copper(II) lactate. Of this compound 8 g were dissolved in 20 ml of water and the solution diluted with 80 ml of dimethylformamide. The solution was slowly added to the zinc oxide dispersion under intensive stirring.

45 The same good results were obtained as in Example 16.

#### EXAMPLE 18

A glassine paper having a weight of 90 g/sq.m was treated in a size-press with the electroconductive aminoalkylated polyethyleneimine of Example 1 and thereafter was calendered to a Bekk surface smoothness of 500-700 (cfr. Wochenschrift fur Papierfabrikation, (June 1957) No. 12, pages 447-451). Both sides of the paper were then covered with a protective layer in a ratio of 7 g/sq.m of a finely ground dispersion formed of zinc oxide and a binding agent. The zinc oxide used was the DIROX (trade-name) variety sold by Vieille Montagne, Belgium, and as binding agent IXAN SGA



was used (trade-name of a copolymer of vinyl chloride, vinylidene chloride, maleic acid, maleic anhydride and acrylonitrile sold by Solvay, Belgium). The weight ratio of zinc oxide pigment to binding agent was 10:4.

900 g of GELVA MULTIPOLYMER solution RP 5 927 A (trade-name) and 2.520 kg Electrographic Resin EO41 (trade-name) were mixed with 10.300 kg of dichloroethane. In the solution obtained 125 g of VIN-NAPAS UW4 (trade-name) were dissolved.

6.300 kg of ELECTROX (trade-name) zinc oxide were dispersed in the above solution under vigorous stirring, whereafter the following sensitizing agents were added:

bromophenol blue as a 1 % solution  
in methanol

93 ml

compound of the formula



as a 0.5 % solution in dimethylformide

104 ml

30

4. An electroconductive substrate according to claim 1, wherein the epihalohydrin is epichlorohydrin.

5. An electroconductive substrate according to claim 1, wherein the organic tertiary amine corresponds to the general formula:



40 wherein:

each of R<sub>1</sub>, R<sub>2</sub>, and R<sub>3</sub> (same or different) represents an alkyl group containing up to 5 carbon atoms, a cycloalkyl group, or an aralkyl group, or R<sub>1</sub>, R<sub>2</sub>, and R<sub>3</sub> together with the nitrogen atom represent a heterocyclic compound.

45 6. An electroconductive substrate according to claim 5, wherein the organic tertiary amine is trimethylamine.

7. An electroconductive substrate according to claim 1, wherein a photoconductive layer is applied to the electroconductive layer to form an electrophotographic recording material.

50 8. An electroconductive substrate according to claim 1, wherein an insulating layer is applied to the electroconductive layer to form an electrographic recording material.

55 9. An electroconductive substrate according to claim 1, wherein the electroconductive layer comprises at least 2 g of aminoalkylated polyethyleneimine per sq.m.

\* \* \* \* \*

To the solution obtained water was added up to a volume of 1 liter.

When the matrix was used in an offset machine very contrasty and sharp copies of the original could be made.

We claim:

1. An electroconductive substrate comprising a support of paper or synthetic polymer, an electroconductive layer coated on at least one side of said support, 60 said electroconductive layer having a surface resistance

measured at 15 % of relative humidity lower than 10<sup>11</sup> ohm/sq., said electroconductive layer consisting of or including a major proportion of an aminoalkylated polyethyleneimine resulting from the reaction at 50°C of epihalohydrin with polyethyleneimine in the presence of an organic tertiary amine, said polymer being soluble in water and becoming insoluble by heating at 100°C.

10 2. An electroconductive substrate according to claim 1, wherein during said reaction of epihalohydrin with polyethyleneimine in the presence of an organic tertiary amine between 0.3 and 1.0 mole of epihalohydrin is present per mole ethyleneimine units in polyethyleneimine, and at least 0.2 mole of organic tertiary amine per mole of epihalohydrin. amine

15 3. An electroconductive substrate according to claim 1, wherein during said reaction 0.4 mole of epihalohydrin is present per mole of ethyleneimine units in polyethyleneimine.

|                                  |       |
|----------------------------------|-------|
| potassium cyanoferrate (II)      | 20 g  |
| potassium cyanoferrate (III)     | 5 g   |
| dipotassium hydrogen phosphate   | 50 g  |
| ethylenediaminetetra-acetic acid | 1 g   |
| glycerol                         | 10 ml |

45

40 wherein:

50 each of R<sub>1</sub>, R<sub>2</sub>, and R<sub>3</sub> (same or different) represents an alkyl group containing up to 5 carbon atoms, a cycloalkyl group, or an aralkyl group, or R<sub>1</sub>, R<sub>2</sub>, and R<sub>3</sub> together with the nitrogen atom represent a heterocyclic compound.

6. An electroconductive substrate according to claim

5, wherein the organic tertiary amine is trimethylamine.

7. An electroconductive substrate according to claim 1, wherein a photoconductive layer is applied to the electroconductive layer to form an electrophotographic recording material.

8. An electroconductive substrate according to claim 1, wherein an insulating layer is applied to the electroconductive layer to form an electrographic recording material.

9. An electroconductive substrate according to claim

1, wherein the electroconductive layer comprises at

least 2 g of aminoalkylated polyethyleneimine per

sq.m.

UNITED STATES PATENT AND TRADEMARK OFFICE  
**CERTIFICATE OF CORRECTION**

PATENT NO. : 3,923,505

DATED : December 2, 1975

INVENTOR(S) : Daniel Maurice Timmerman et al

It is certified that error appears in the above-identified patent and that said Letters Patent are hereby corrected as shown below:

In the Title: The last word of the title should be corrected to read: -- Polyethyleneimine --.

Item [30] Foreign Application Priority Data:

"June 16, 1972 Germany 028432" should read

-- June 16, 1972 Great Britain 028423 --.

In the Claims: Column 16, line 13, after "mole" insert -- of --; line 15, delete "amine" after the period.

Signed and Sealed this  
second Day of March 1976

[SEAL]

Attest:

**RUTH C. MASON**  
Attesting Officer

**C. MARSHALL DANN**  
Commissioner of Patents and Trademarks